

## UNITED STATES PATENT OFFICE

2,092,686

## METHOD OF POLISHING WAX

Mack Wilson, Washington, D. C., assignor of one-half to Joseph E. Stacey, Dorchester, Mass.

No Drawing. Application March 16, 1937,  
Serial No. 131,269

## 10 Claims.

(Cl. 91—68)

This invention relates to the treatment of wooden, metallic, leather or other surfaces by waxing and polishing the same, and more particularly to a method of imparting a satisfactory 5 polish to the wax used in treating such surfaces.

In waxing furniture, floors, automobile bodies, leather goods and other surfaces to which wax may be applied in either liquid, cream or paste form, it has heretofore been necessary (except in 10 the case of the so-called self-polishing waxes) to expend considerable energy in rubbing the wax, either manually or by machine, in order to produce the hard, bright finish or polish desired. For example, it is well known that in polishing 15 automobile bodies by far the greatest portion of the time and labor required is utilized in polishing the wax after it is applied. Not only is this polishing operation a long and laborious one, but it also results in the actual removal by the polishing cloth or other instrument from the surface being treated of a substantial amount of the wax originally applied, leaving the surface with a thinner layer of wax thereon than might otherwise be obtained. The wax thus removed is not 20 only wasted but also contaminates the cloth or other polisher making it necessary to replace or clean the same at frequent intervals:

It is therefore one of the objects of the present invention to provide a novel method of polishing wax as applied to various kinds of surfaces which 25 will effect a substantial saving in the time, labor and expense involved in producing the fine, high gloss or luster desired.

Another object is to provide an improved procedure for waxing and polishing surfaces which 30 will leave on the surface in polished form a greater proportion of the amount of wax applied thereto than remains after the mere rubbing operation heretofore practiced, and which therefore 35 requires less wax for the same thickness of coat and less frequent replacement or cleaning of the polishing utensils.

A further object is to provide a new method of bringing waxed surfaces to a bright polish which 40 is not only quicker, less laborious and less expensive, but also produces a finer and more lasting finish, than the procedures previously followed.

It has been discovered that these and other 45 objects, which will appear more fully upon consideration of the following description of the invention, may be attained by a procedure which is characterized primarily by the use of a dry, comminuted or powdered material of the vegetable kingdom as the wax polishing agent.

50 Although other finely divided materials may

function to some degree as wax polishing agents, it has been found that the desired results are best attained by the use of a flour, meal or powdered starch formed from one or more of the group of 5 vegetable substances comprising wheat, corn, rye, barley, oats, potatoes and wood. In using the term "flour" as applied to these substances it is intended to include the pulverized fibrous constituents thereof as well as the finely ground 10 starchy constituents; for example, powdered wood, such as results from a sanding operation thereof, and pulverized straw are both suitable for use in the present method. Of these various substances, however, wheat flour, corn flour and 15 corn starch, either separately or any combination thereof, are preferred. Excellent results have been obtained by the use of a powder consisting entirely of a high grade wheat flour. While these substances may be used in their ordinary 20 powdered state with full effect as far as their polishing action is concerned, it is often desirable for commercial reasons to add to the powder suitable quantities of coloring and flavoring or perfume substances.

In carrying out the method of the present invention, the surface to be treated is first coated with wax in the usual manner, it being understood that any suitable liquid, cream or paste 25 polishing wax may be used, other than a self-polishing wax. Immediately after application of the wax, a small quantity of comminuted or powdered polishing material is sprinkled over the wax and also upon a cloth or other suitable polishing instrument which is then used to rub the powder 30 over the wax until the desired degree of polish is obtained. The powder is then removed in any suitable manner as by dusting with a clean cloth, 35 an air blast or a vacuum cleaner.

The exact manner in which the powder functions to produce the unusually fine polish resulting 40 from this procedure is not known, although it has been observed that very little wax is removed from the surface being treated during the polishing operation and that whatever amount is removed does not appear to be absorbed by or 45 deposited on the cloth or other polishing instrument to any noticeable extent. In this connection, it has been found that the polishing operation of the present method may be carried out not only by the use of any of the known polishing 50 instruments, such as cloths, woolen polishers, polisher mitts and polisher machines, but also by employing soft paper or even the human hand; this result is apparently due to the fact that the 55 polishing instrument, whatever it may be, serves

only as a carrier for the powder which is the real polishing agent.

In using the powdered polisher as above described, a relatively light coat thereof sprinkled over the wax will ordinarily suffice; for example, five ounces of a high grade wheat flour powder will polish the wax on the surfaces of eight average sized automobile bodies or an equivalent area of other surfaces. Although the method of the present invention requires an expenditure for the powder used, the savings effected in the cost of labor and polishing materials far exceed the added cost of the powder. As a result of time studies made at a number of automobile service stations, it has been established that the present method saves between 50% and 75% of the time required for polishing wax, and at the same time enables the work to be done with far less expenditure of energy since under ordinary conditions a relatively light rubbing is all that is required. Another advantage of this method is that it is possible thereby to bring wax to a polish even though it has become dry before the polishing operation is begun, whereas this is practically impossible of accomplishment by the ordinary method of merely rubbing the wax with a cloth or the like.

There is thus provided by the present invention a novel and highly useful method of polishing wax which is quicker, easier, less expensive and productive of better results than the procedures heretofore employed for the same purpose. While the method of the invention is particularly well adapted to the polishing of automobile bodies, it is equally useful in the treatment of all kinds of surfaces to which wax may be applied, such as floors, furniture, woodwork, linoleum, machinery, shoes and other leather and imitation leather articles. Likewise, it will be obvious that the invention is applicable to the polishing of all kinds of waxes, whether liquid, cream or paste, excluding only the so-called self-polishing waxes.

In the foregoing description of the invention a number of different substances have been specified as useful in forming the powdered polishing agent employed in the method. While all of these substances have been tested and found operative, it is realized that there may be other materials which are also capable of use and should be included within the scope of the invention. It should also be recognized that the manner in which the polishing powder is applied to and rubbed over the wax is subject to variation without exceeding the limits of the invention; for example, it is contemplated that the powder may be marketed in a cloth bag, rather than in an ordinary can or other container, and that the bag may serve both as the source of powder and as the instrument by which the powder is rubbed over the wax to effect the polishing. Various other modifications, which will now occur to those skilled in the art, may be made in the details of procedure and means employed in practicing the same without departing from the spirit of the invention. Reference is therefore to be had to the appended claims for a definition of the scope of the invention.

What is claimed is:

1. A method of polishing surfaces by the use of wax comprising the steps of applying a coating of wax to the surface to be treated, applying to the surface of the wax a dry, comminuted vegetable material, and then rubbing the said mate-

rial over the surface of the wax until the desired polish is produced.

2. A method of polishing surfaces by the use of wax comprising the steps of applying a coating of wax to the surface to be treated, applying to the surface of the wax a powder the ingredients of which are selected from the group of vegetable substances consisting of wheat, corn, rye, barley, oats, potatoes and wood, and then rubbing the said powder over the surface of the wax until the desired polish is produced.

3. A method of polishing surfaces by the use of wax comprising the steps of applying a coating of wax to the surface to be treated, applying to the surface of the wax a flour or meal formed from one or more of the group of vegetable substances consisting of wheat, corn, rye, barley, oats, potatoes and wood, and then rubbing the said flour or meal over the surface of the wax until the desired polish is produced.

4. A method of polishing surfaces by the use of wax comprising the steps of applying a coating of wax to the surface to be treated, applying to the surface of the wax a pulverized fibrous vegetable material, and then rubbing the said material over the surface of the wax until the desired polish is produced.

5. A method of polishing surfaces by the use of wax comprising the steps of applying a coating of wax to the surface to be treated, coating the surface of said wax with a pulverized woody material, and then rubbing the said material over the surface of the wax until the desired polish is produced.

6. A method of polishing surfaces by the use of wax and a polishing instrument such as a cloth comprising the steps of applying a coating of wax to the surface to be treated, applying to the surface of the wax a coating of comminuted vegetable material, applying a similar coating of said material to the polishing instrument, and then rubbing the coated instrument over the coated surface of the wax until the desired polish is produced.

7. A method of polishing surfaces by the use of wax and a polishing instrument such as a cloth comprising the steps of applying a coating of wax to the surface to be treated, applying to the surface of the wax a coating of comminuted vegetable material, applying a similar coating of said material to the polishing instrument, rubbing the coated instrument over the coated surface of the wax until the desired polish is produced, and then removing from the polished surface of the wax whatever amount of said material remains thereon.

8. A method of imparting a polish to wax comprising the steps of coating the surface of the wax with a dry, finely divided vegetable material, and then rubbing the said material over the surface of the wax until the desired polish is produced.

9. A method of imparting a polish to wax comprising the steps of sprinkling the surface of the wax with a powdered starchy material, and then rubbing the said material over the surface of the wax until the desired polish is produced.

10. A method of imparting a polish to wax comprising the steps of coating the surface of the wax with wheat flour, applying a coating of said flour to a polishing instrument such as a cloth, and then rubbing the coated instrument over the coated surface of the wax until the desired polish is produced.

MACK WILSON.